

## UNITED STATES PATENT OFFICE

2,177,751

## ENGRAVING PROCESS

Edward A. Sikorski, Parma, Ohio, assignor to  
 General Chemical Company, New York, N. Y.,  
 a corporation of New York

No Drawing. Application May 28, 1938,  
 Serial No. 210,775

6 Claims. (Cl. 41—42)

This invention relates to the art of engraving or etching metals. More particularly, the invention is directed to improvements in processes for etching metals and in metal etching baths.

5 The general procedure involved in the engraving or etching of metals such as steel, copper and zinc is well known. Briefly, the metal to be etched is covered with a ground of acid-resistant material such as varnish, wax or resin. 10 The design to be etched is made on the surface of the metal by cutting away or otherwise removing part of the ground. The metal is then subjected to the action of an acid bath which bites out exposed or uncovered parts of the metal. The 15 bath usually employed is a water solution containing around 10% nitric acid.

Several suggestions have been made as to addition to the nitric acid of small amounts of other substances for the purpose of improving the properties of the nitric acid principally with respect to "bite", non-discoloration of the bath and of the work, and to impart to the bath a longer life. While some progress has been made, the materials previously suggested have been such as to bring about improvements with respect to one or another but not all of the important properties a satisfactory etching process and etching bath should have. Another difficulty is that in many instances prior proposals have required 20 introduction into the nitric acid of materials which raise the impurity content of the acid above the amounts permissible in recognized trade specifications.

I have found that the etching process may be 25 made much more efficient if carried out in the presence of a small amount of urea and I have discovered that addition of a small amount of urea to the nitric acid substantially enhances the value of the acid with respect to each of the 30 desirable properties an etching bath should possess. While lesser amounts may be used, more specifically I have found that much improved results may be obtained by carrying out the etching process in a bath containing nitric acid and 35 urea, the acid and urea being in the proportion of not less than 0.3 part by weight of urea per 100 parts by weight of nitric acid, 100% basis. I prefer to use nitric acid and urea in proportion of about 0.32 part by weight of urea per 100 parts 40 by weight of 100% nitric acid. Greater amounts of urea may be employed to no disadvantage.

As stated, the nitric acid concentration of most customary commercial etching baths is about 45 10%. If desired the urea in proper amount may be added directly to the relatively dilute etching

bath. However, it is more convenient and usually more desirable to first incorporate the urea with the stronger nitric acid usually available on the market in concentrations ranging from 38 to 42° Bé. In practicing the invention, the strong nitric acid containing the indicated amounts of urea is diluted with water in quantity to form a bath having the customary 9-10% or other suitable nitric acid concentration. In some types of operation, the bath is much stronger, and in some 10 particular instances the  $\text{HNO}_3$  concentration of the bath may be as high as 30-32° Bé. or more, depending upon the action desired.

The bath is fed into an open rocker, splasher-type or other common etching machine. The 15 metal to be etched is then subjected to the action of the bath for example by immersion or splashing. The technique employed is variable depending upon the type of work, depth of cut desired, time of treatment, and other factors and is well 20 understood in the etching art. The temperature of the bath is preferably kept at about 70° F., and usually not permitted to exceed about 80° F.

I have found that by carrying out the process 25 as described discoloration of the work is prevented. The bath remains substantially water white or very slightly yellow. Little fuming of nitrogen oxides occurs. The work is clean-cut, and etched lines and dots are sharp. Addition of a small amount of urea to the acid substantially 30 lengthens the effective life of the bath. Further, experience shows that the rate and degree of "bite" are materially improved.

The reasons why the improved results are obtained are not understood. It is known that 35 attack of nitric acid on various metals yields nitric oxide ( $\text{NO}$ ), nitrogen tetroxide ( $\text{NO}_2$ ), or even  $\text{NH}_3$  or other oxides of nitrogen depending upon conditions such as the metal treated, concentration of the acid, temperatures, etc. The 40 reaction of nitric acid with metals is complicated, usually slow at first and increasing in speed with accumulation of reduction products. The chemical reactions taking place in etching operations are dependent upon many different factors, 45 are very complex and very little is definitely known of the exact nature of such reactions. In all etching processes there seems to be a tendency toward formation of free oxides of nitrogen including the brown  $\text{NO}_2$ . In the process of the 50 invention, with urea present it appears that the oxides of nitrogen such as  $\text{NO}$  and  $\text{NO}_2$  are largely acted upon by urea in some complex way to form gaseous nitrogen and water and possibly some 55  $\text{NH}_3$ . It definitely appears, however, that the

process of urea inhibits production of fume-forming nitrogen oxides, and such inhibiting action evidently contributes in some way or other, possibly catalytically, to increase the bite of the acid and extend the life of the bath.

5 I claim:

1. The process for etching metal which comprises subjecting the metal to the action of an etching bath comprising nitric acid having incorporated therewith a small amount of urea.
- 10 2. The process for etching metal which comprises subjecting the metal to the action of an etching bath comprising nitric acid having incorporated therewith urea in the proportion of not less than 0.3 part by weight of urea per 100 parts by weight of nitric acid, 100% basis.
- 15 3. The process for etching metal which com-

prises subjecting the metal to the action of an etching bath comprising nitric acid having incorporated therewith urea in the proportion of about 0.32 part by weight of urea per 100 parts by weight of nitric acid, 100% basis.

4. An etching bath comprising nitric acid having incorporated therewith a small amount of urea.

5. An etching bath comprising nitric acid having incorporated therewith urea in the proportion of not less than 0.3 part by weight of urea per 100 parts by weight of nitric acid, 100% basis.

6. An etching bath comprising nitric acid having incorporated therewith urea in the proportion of about 0.32 part by weight of urea per 100 parts by weight of nitric acid, 100% basis.

EDWARD A. SIKORSKI.